

**1**

2,931,835

**QUATERNARY PHOSPHONIUM POLYPHOSPHATES**

Peter William Brett Semmens, Norton-on-Tees, England, assignor to Imperial Chemical Industries Limited, London, England, a corporation of Great Britain

No Drawing. Application April 9, 1956  
Serial No. 576,758

Claims priority, application Great Britain April 20, 1955

6 Claims. (Cl. 260—606.5)

This invention relates to quaternary phosphonium polyphosphate compounds which are new compounds.

According to the present invention, there is provided a quaternary phosphonium polyphosphate salt having  $(\overline{\text{PO}}_3)^-$  units forming substantially linear groups, each  $(\overline{\text{PO}}_3)^-$  unit being associated with a cation, a major proportion of such cations being quaternary phosphonium cations, in each of which the four valences of the phosphorus ion are attached to organic radicals.

The organic radicals in each quaternary phosphonium group may be all alike, or some or all may be different, and they may comprise alkyl, aryl, aralkyl, or alicyclic groups, or substituted derivatives thereof.

There may also be a minor proportion of sodium, potassium or other cations associated with the  $(\overline{\text{PO}}_3)^-$  units. These cations may be present as a result of their incomplete substitution in a polyphosphate salt by quaternary phosphonium cations, or they may be deliberately introduced during the preparation of the compounds of the present invention. In a preferred group of polyphosphate compounds of the present invention at least one of said organic radicals includes at least one alkyl radical having six or more carbon atoms. Such organic radicals include for example octyl, decyl, dodecyl, tetradecyl, cetyl and lauryl, and radicals such as beta-para-tert.-octyl phenoxyethyl in which the alkyl radical having the required minimum number of carbon atoms forms part of a larger radical which may include other alkyl or aryl radicals, and/or other functional groups. The preferred polyphosphate compounds of the present invention include for example, cetyl tripropyl phosphonium polyphosphate, didecyl dimethyl phosphonium polyphosphate and tetra-decyl phosphonium polyphosphate.

According to a further feature of the present invention new compositions of matter are provided which are suitable for use as boundary lubricants and which comprise one or more of the preferred polyphosphate compounds of this invention dissolved or dispersed in a liquid or solid vehicle which is preferably a lubricant. Suitable vehicles which are lubricants include for example, mineral or vegetable oils or greases, esters of aliphatic dicarboxylic acids, polyalkylene glycols, polymethyl-phenyl siloxanes, mixtures of substantially completely halogenated aromatic hydrocarbons such as that sold under the British registered trademark "Florube" 1, or any combination of these. The relative proportions of vehicle in these compositions may be varied over a wide range.

**2**

The polyphosphate compounds of the present invention may be used as insecticides or to give water repellent finishes to glass or textiles.

The preferred polyphosphate compounds of this invention provide effective boundary lubricants of ferrous metals and may be used either alone or in admixture with suitable materials. Boundary lubricants are effective in lubricating surfaces, particularly metal surfaces, which are sliding under conditions of heavy loads and/or slow relative sliding speeds, these conditions usually being known as boundary conditions. Under boundary conditions, surface contact occurs and frictional forces between sliding surfaces are considerable, resulting in wear and even, in extreme cases, in seizure of the sliding parts. 10 The effectiveness of these preferred compounds as boundary lubricants is therefore a most important property. They are effective boundary lubricants of mild steel surfaces and of austenitic stainless steel surfaces such as austenitic stainless steel shafts in journal bearings. 15 Potassium polyphosphate for use in the process of the present invention may be prepared by heating potassium dihydrogen orthophosphate at a suitable temperature, for example 650° to 700° C., for a period of preferably about one hour. 20 Solubilised polyphosphates suitable for use in the process of the present invention may be produced by any of the following methods: 25 (a) Powdered potassium polyphosphate may be added to water, and contacted with the sodium salt of a cation exchange resin, such as, for example, the sodium salt of a sulphonated polystyrene or of a sulphonated phenolic resin. The potassium polyphosphate, on treatment in this manner, goes into solution as a sodium-potassium polyphosphate. 30 (b) Instead of using a sodium salt of a cation exchange resin as described in (a), it is possible to use an ammonium salt of a cation exchange resin. On treatment in this manner the potassium polyphosphate goes into solution as ammonium-potassium polyphosphate. 35 (c) The use of the salt of a cation exchange resin as in (a) and (b), has the disadvantage that the resin must either be discarded or regenerated. An alternative method which avoids the use of a cation exchange resin is to allow powdered potassium polyphosphate to stand in contact with a solution of a sodium salt, for example sodium chloride. The product swells during this treatment, and may be dissolved in water to give a viscous solution suitable for use in the process of the present invention. 40 (d) Potassium polyphosphate is solubilised on treatment with hydrogen peroxide, for example by adding potassium polyphosphate to hydrogen peroxide. It is necessary to neutralise the hydrogen peroxide, which usually contains a small quantity of acid, prior to use by the addition of a small quantity of alkali.

45 The solubilised potassium polyphosphate is brought into contact in solution with an aqueous solution of quaternary phosphonium salt, such as the bromide, for example by mixing with stirring. It is preferred to add the phosphonium salt solution gradually, and to stop when precipitation of the quaternary phosphonium polyphosphate, which comes out of solution during the addition, is complete. The concentrations of the polyphosphate solution and the quaternary phosphonium salt solution are not critical, but it is preferred that they should be

approximately equal and approximately 1% by weight. The product may then be separated, washed with water and dried.

As an alternative to first solubilising potassium polyphosphate, the products of the present invention may be prepared by bringing powdered potassium polyphosphate into contact with an aqueous solution of quaternary phosphonium salt, for example the bromide. The product swells during this treatment, and may be washed to remove excess quaternary phosphonium salt and potassium halide.

The quaternary phosphonium polyphosphates of the present invention are in general solids which are insoluble in water, but they may be soluble in organic solvents such as chloroform.

#### EXAMPLE 1

120 grams of air dried ion exchange resin sold under the British registered trademark "Zeo-Karb 215" were activated into the ammonium form by treatment with ammonium chloride. The exchange resin was then washed free from chloride ions and added to sufficient water to give a total volume of 600 mls. 9 grams of potassium polyphosphate were added and the mixture stirred in the cold for 45 minutes, after which the temperature was slowly raised to 50° C. when complete solution occurred. After removing the resin by filtration, the resulting solution had the following analysis:

|                                                   | Percent by weight |
|---------------------------------------------------|-------------------|
| P <sub>2</sub> O <sub>5</sub> as KPO <sub>3</sub> | 1.58              |
| NH <sub>4</sub>                                   | 0.2               |
| K                                                 | 0.1               |

Coefficient of friction between austenitic stainless steel surfaces—surface speed 0.08 cm./sec.

| Lubricant              |                 | Coefficient of friction |        |         |         |         |         |         |         |
|------------------------|-----------------|-------------------------|--------|---------|---------|---------|---------|---------|---------|
| Percent Poly-phosphate | Percent vehicle | 20° C.                  | 60° C. | 100° C. | 120° C. | 140° C. | 160° C. | 180° C. | 200° C. |
| NH                     | NH              | 1.11                    | 1.27   | 1.24    | 1.30    | 1.28    | 1.25    | 1.28    | 1.31    |
| NH                     | 100% MO         | 0.12                    | 0.12   | 0.12    | 0.12    | 0.13    | 0.16    | 0.18    | 0.20    |
| 5% CPP                 | 95% MO          | 0.11                    | 0.11   | 0.09    | 0.08    | 0.08    | 0.08    | 0.07    | 0.12    |
| NH                     | 100% DS         | 0.14                    | 0.15   | 0.18    | 0.18    | 0.19    | 0.21    | 0.23    | 0.23    |
| 5% CPP                 | 95% DS          | 0.12                    | 0.10   | 0.10    | 0.08    | 0.08    | 0.07    | 0.08    | 0.08    |
| NH                     | 100% PAG        | 0.15                    | 0.21   | 0.21    | 0.20    | 0.19    | 0.22    | 0.20    | 0.23    |
| 5% CPP                 | 95% PAG         | 0.14                    | 0.12   | 0.10    | 0.09    | 0.09    | 0.10    | 0.12    | 0.12    |
| NH                     | 100% CX         | 0.15                    | 0.15   | 0.16    | 0.17    | 0.19    | 0.17    | 0.20    | 0.18    |
| 5% CPP                 | 95% CX          | 0.14                    | 0.12   | 0.10    | 0.10    | 0.11    | 0.11    | 0.10    | 0.10    |
| NH                     | 100% PPS        | 0.20                    | 0.20   | 0.26    | 0.43    | 0.53    | 0.01    | 0.87    | 0.98    |
| 5% CPP                 | 95% PPS         | 0.16                    | 0.16   | 0.21    | 0.17    | 0.23    | 0.23    | 0.23    | 0.23    |
| 100% CPP               | NH              | 0.08                    | 0.06   | 0.06    | 0.06    | 0.05    | ---     | ---     | ---     |

References:

MO—Mineral oil, viscosity 350 cs. at 70° F., 12 cs. at 200° F.

DS—D(ethyl hexyl) sebacate.

PAG—Polyalkylene glycol, viscosity 61.7 c.s. at 100° F., 11 c.s. at 210° F.

CX—"Florube" 1, (British registered Trademark).

PPS—Polymethyl-phenyl siloxane, viscosity 250 cs. at 100° F., 25 cs. at 210° F.

CPP—Cetyl tripropyl phosphonium polyphosphate.

This was diluted to give a 1% solution by weight calculated as KPO<sub>3</sub>, and to 50 mls. of this solution a 1% by weight aqueous solution of cetyl tripropyl phosphonium bromide was added with stirring until the precipitation of cetyl tripropyl phosphonium polyphosphate was complete. This occurred when approximately 185 mls. of the cetyl tripropyl phosphonium bromide solution had been added. The product was separated by filtration, washed in water and dried in an oven at 185° C.

#### EXAMPLE 2

2.5 grams of potassium polyphosphate were added to 50 mls. of a solution containing sufficient sodium chloride to give a potassium:sodium atomic ratio of 1:2. The mixture was slowly stirred for 1/4 hour, the solution poured off and 180 mls. of water added. After rapid agitation, nearly all of the swollen residue passed into solution. A small amount of undissolved material was separated by filtration. 50 mls. of this solution were treated in the same way as in Example 1 by the addition

of a 1% aqueous solution of cetyl tripropyl phosphonium bromide. The product was collected in the same way as in Example 1.

#### EXAMPLE 3

200 mls. of 29% w./v. hydrogen peroxide diluted with 200 mls. of water were neutralised with 2 mls. of normal sodium hydroxide solution, and added to 8 grams 10 of potassium polyphosphate. The mixture was vigorously 15 stirred and after 15 minutes the potassium polyphosphate was completely dissolved. A further 350 mls. of water were added to the solution which then contained 1% by weight of KPO<sub>3</sub>. 50 mls. of this solution were treated as in Examples 1 and 2.

Cetyl tripropyl phosphonium polyphosphate was tested as a boundary lubricant in the following way. Coefficients of friction were measured between 20° and 200° C. on a kinetic boundary friction apparatus, the moving surfaces being of austenitic stainless steel and moving at a relative speed of 0.08 cm. per second. Measurements were made using no lubricant and using vehicles only as lubricants. Further measurements were made using cetyl tripropyl phosphonium polyphosphate alone as a lubricant, and also in the form of a 5% dispersion by weight in the vehicles tested.

The results obtained are given in the table below.

The dispersions tested were made by mixing the two components by stirring, if necessary with heating to moderate temperatures for a short time.

Coefficient of friction between austenitic stainless steel surfaces—surface speed 0.08 cm./sec.

It will be seen that the vehicle-polyphosphate compositions are effective boundary lubricants and even at a concentration as low as 5%, there is an improvement over the vehicle used alone which becomes more marked 60 at higher temperatures. It can further be seen that the effectiveness of the compositions in most cases is maintained over a wide temperature range.

I claim:

1. A quaternary phosphonium polyphosphate salt having (PO<sub>3</sub>)<sup>-</sup> units forming substantially linear groups, each (PO<sub>3</sub>)<sup>-</sup> unit being associated with a cation, the major proportion of such cations being quaternary phosphonium cations, in each of which the four valences of the phosphorous atom are attached to organic radicals selected from the group consisting of alkyl radicals and monocyclic aryloxyalkyl groups and the minor proportion of such cations being selected from the group consisting of hydrogen, ammonium, sodium and potassium ions.

70 2. A quaternary phosphonium polyphosphate salt as

set forth in claim 1 in which the organic radical is a beta-p-tertiaryoctylphenoxyethyl radical.

3. A compound according to claim 1 in which at least one of said organic radicals includes at least one alkyl radical having at least six carbon atoms.

4. A compound according to claim 1 in which the said quaternary phosphonium cations are cetyl tripropyl phosphonium groups.

5. A compound according to claim 1 in which the said quaternary phosphonium cations are didecyl dimethyl phosphonium groups. 10

6. A compound according to claim 1 in which the said

quaternary phosphonium cations are tetradecyl phosphonium groups.

References Cited in the file of this patent

UNITED STATES PATENTS

|           |           |       |               |
|-----------|-----------|-------|---------------|
| 2,220,851 | Schreiber | ----- | Nov. 5, 1940  |
| 2,360,623 | Rosen     | ----- | Oct. 17, 1944 |
| 2,414,263 | Kemp      | ----- | Jan. 14, 1947 |
| 2,446,647 | Stern     | ----- | Apr. 5, 1949  |
| 2,703,814 | Dye       | ----- | Mar. 8, 1955  |
| 2,745,877 | Binder    | ----- | May 15, 1956  |